

## UNITED STATES PATENT OFFICE

2,552,229

FOG INHIBITORS FOR PHOTOGRAPHIC  
EMULSIONS

Robert E. Stauffer and William F. Smith, Rochester, N. Y., assignors to Eastman Kodak Company, Rochester, N. Y., a corporation of New Jersey

No Drawing. Application May 4, 1949,  
Serial No. 91,426

11 Claims. (Cl. 95—7)

1

This invention relates to fog-inhibiting agents and stabilizers for photographic emulsions and to photographic emulsions containing them.

It is known that photographic emulsions, particularly ultra-sensitive emulsions or those containing optical sensitizers exhibit a tendency to form a deposit of silver in the emulsion. This deposit extends more or less uniformly over the entire emulsion and is known as fog. Photographic fog is of two types: local and general. Local fog is formed by exposure of the film or plate at undesired points as by a light leak in the camera. General fog is formed in a number of ways. It may be caused by the conditions under which the film or plate is stored such as conditions of high temperature or humidity or unusually long time of storage. The nature of the emulsion may also produce general fog as well as the conditions of development of the emulsion as by development for protracted periods of time or at temperatures above normal. We are primarily concerned with the fog and sensitivity changes in films or plates which have been stored under adverse conditions of temperature and humidity.

General fog and loss of sensitivity of the emulsion are especially likely to occur when the sensitive material is stored under conditions other than ideal, that is, under conditions of high temperature and humidity as in tropical regions.

It is an object of the invention to provide novel anti-fogging or fog-inhibiting compounds for emulsions. A further object is to provide anti-fogging agents which stabilize the initial sensitivity of the emulsion. A still further object is to provide anti-fogging agents which improve the keeping of the emulsion in tropical regions. Other objects will appear from the following description of our invention.

These objects are accomplished by incorporating into a silver halide emulsion a palladous salt complex as a stabilizing agent. The following compounds are given as examples of the compounds useful in our invention.

Diethylenediammine palladous chloride,  
 $Pd(H_2NC_2H_4NH_2)_2Cl_2$   
 Ethyldiamminepalladous chloride,  $Pd(C_2H_5NH_2)_2Cl_2$   
 Dipyridiniumpalladous chloride,  $Pd(C_6H_5N)_2Cl_2$   
 Diamminepalladous chloride,  $Pd(NH_3)_2Cl_2$   
 Diquinoliniumpalladous chloride,  $Pd(C_6H_7N)_2Cl_2$

2

Benzylidiamminepalladous chloride,  $Pd(C_6H_5N)_2Cl_2$   
 Diethylenepalladous chloride,  $Pd(C_2H_4)_2Cl_2$   
 Diamminepalladous bromide,  $Pd(NH_3)_2Br_2$   
 Diamminepalladous iodide,  $Pd(NH_3)_2I_2$   
 Diamminepalladous sulfate,  $Pd(NH_3)_2SO_4$   
 Diamminepalladous carbonate,  $Pd(NH_3)_2CO_3$   
 Diamminepalladous nitrate,  $Pd(NH_3)_2(NO_3)_2$

These compounds are described in the Textbook of Inorganic Chemistry by M. M. J. Sutherland, published by Charles Griffin and Company, Ltd., London, vol. 10, pp. 193-243 (1928), and may be called acido-palladium compounds or complexes in which the basic compounds, or ethylene, exists in the cation strongly bonded to the palladium atom and the anion of the complex is a mono-valent or di-valent anion of an acid. As is apparent the useful compounds include the complexes in which the group bound to the palladium atom is either ethylene, ammonia or an organic base, e. g., methyl, ethyl, propyl or iso-propylamines, heterocyclic tertiary nitrogen compounds as quinoline and pyridine; benzylamine or ethylene diamine. The anion of the complex may, for example, be either halide, sulfate, carbonate or nitrate.

25 The object of our invention is to maintain the sensitivity and fog of silver halide emulsions at or close to initial optimum values under keeping conditions of high temperature and humidity. The fog inhibitors which we propose to use are added to the emulsion during the process of manufacture to avoid loss of sensitivity and to inhibit the growth of fog with passage of time under non-ideal conditions of storage.

30 A solution of the compounds of the invention when added in suitable concentration before coating to unsensitized or optically sensitized photographic emulsions does not appreciably affect the sensitometric values for sensitivity and fog when measurements are made soon after coating. When sensitometric measurements are 35 made at appreciable intervals of time under tropical or dry conditions of storage at elevated temperatures, however, these compounds do stabilize photographic speed and maintain fog at a low level.

40 The preparation of silver halide emulsions involves three separate operations (1) the emulsification and digestion or ripening of the silver halide, (2) the freeing of the emulsion from excess soluble salts usually by washing, (3) the 45 second digestion or after-ripening to obtain in-

creased sensitivity. (Mees, The Theory of the Photographic Process, 1942.) We prefer to add the fog-inhibiting agents after the final digestion or after-ripening although they may be added before digestion. The most useful concentration range of fog inhibitor is from .26 to 3.9 gm. of fog inhibitor per kilogram of silver nitrate used in making the particular silver halide emulsion and converted to silver halide. The quantity used will of course vary for example depending on the silver halide or mixture of halides used

5 used a high-speed silver bromoiodide emulsion exposed on an Eastman type IB sensitometer and developed for five minutes in a developer of the following composition:

|                                    | Grams |
|------------------------------------|-------|
| Monomethyl paraaminophenol sulfate | 2.5   |
| Sodium sulfite (desiccated)        | 30    |
| Hydroquinone                       | 2.5   |
| Sodium metaborate                  | 10    |
| Potassium bromide                  | 0.5   |
| Water to one liter.                |       |

| Sample No. | Gms. of compound per Kg. AgNO <sub>3</sub> (converted to AgX) in emulsion | Conditioned to 45% R. H. |       |      |                |       |     |     |
|------------|---------------------------------------------------------------------------|--------------------------|-------|------|----------------|-------|-----|-----|
|            |                                                                           | Original                 |       |      | 18 da. 120° F. |       |     |     |
|            |                                                                           | 1/i Speed                | Gamma | Fog  | 1/i Speed      | Gamma | Fog |     |
| 1          | Control                                                                   | None                     | 105   | .98  | .03            | 49    | .82 | .21 |
| 2          | Pd(NH <sub>3</sub> ) <sub>2</sub> Br <sub>2</sub>                         | 0.50                     | 108   | .95  | .03            | 84    | .87 | .07 |
| 3          | Pd(NH <sub>3</sub> ) <sub>2</sub> Br <sub>2</sub>                         | 1.00                     | 98    | .98  | .02            | 90    | .95 | .07 |
| 4          | Pd(NH <sub>3</sub> ) <sub>2</sub> Br <sub>2</sub>                         | 1.50                     | 94    | .98  | .02            | 92    | .93 | .05 |
| 5          | Pd(NH <sub>3</sub> ) <sub>2</sub> I <sub>2</sub>                          | 0.50                     | 96    | .95  | .03            | 76    | .94 | .08 |
| 6          | Pd(NH <sub>3</sub> ) <sub>2</sub> I <sub>2</sub>                          | 1.00                     | 92    | .99  | .04            | 82    | .98 | .05 |
| 7          | Pd(NH <sub>3</sub> ) <sub>2</sub> I <sub>2</sub>                          | 1.50                     | 94    | 1.07 | .02            | 80    | .98 | .06 |
| 8          | Control                                                                   | None                     | 115   | .97  | .04            | 76    | .88 | .10 |
| 9          | Pd(NH <sub>3</sub> ) <sub>2</sub> Cl <sub>2</sub>                         | 0.50                     | 110   | .97  | .02            | 94    | .90 | .06 |
| 10         | Pd(NH <sub>3</sub> ) <sub>2</sub> Cl <sub>2</sub>                         | 1.00                     | 105   | 1.01 | .02            | 88    | .89 | .07 |
| 11         | Pd(NH <sub>3</sub> ) <sub>2</sub> Cl <sub>2</sub>                         | 1.50                     | 100   | .97  | .02            | 88    | .89 | .09 |

| Sample No. | Conditioned to 60% R. H. |       |     |                |       |     | Conditioned to 70% R. H. |       |     |               |       |     |
|------------|--------------------------|-------|-----|----------------|-------|-----|--------------------------|-------|-----|---------------|-------|-----|
|            | Original                 |       |     | 18 da. 120° F. |       |     | Original                 |       |     | 6 da. 120° F. |       |     |
|            | 1/i Speed                | Gamma | Fog | 1/i Speed      | Gamma | Fog | 1/i Speed                | Gamma | Fog | 1/i Speed     | Gamma | Fog |
| 1          | 100                      | 1.02  | .02 | 39             | .77   | .30 | 110                      | 1.02  | .02 | 73            | .90   | .06 |
| 2          | 110                      | 1.00  | .02 | 76             | .87   | .07 | 100                      | .97   | .03 | 65            | .85   | .09 |
| 3          | 98                       | 1.02  | .02 | 68             | .88   | .08 | 98                       | 1.01  | .03 | 63            | .87   | .10 |
| 4          | 100                      | 1.03  | .01 | 88             | .98   | .05 | 96                       | 1.04  | .04 | 55            | .92   | .09 |
| 5          | 96                       | 1.08  | .02 | 61             | .91   | .09 | 100                      | 1.01  | .03 | 65            | .98   | .07 |
| 6          | 100                      | 1.09  | .02 | 52             | .90   | .11 | 92                       | 1.02  | .03 | 65            | .98   | .07 |
| 7          | 92                       | 1.12  | .02 | 66             | .89   | .08 | 105                      | .94   | .03 | 24            | .80   | .38 |
| 8          | 110                      | .96   | .02 | 37             | .75   | .24 | 100                      | 1.01  | .05 | 53            | .84   | .15 |
| 9          | 110                      | .98   | .02 | 65             | .87   | .10 | 105                      | 1.00  | .03 | 63            | .86   | .10 |
| 10         | 100                      | .99   | .02 | 82             | .86   | .08 | 100                      | 1.01  | .02 | 59            | .87   | .12 |
| 11         | 98                       | .99   | .02 | 88             | .86   | .07 | 100                      | 1.01  | .02 | 59            | .87   | .12 |

| Sample No. | Gms. of compound per Kg. AgNO <sub>3</sub> (converted to AgX) in emulsion                         | Original   |       |      | 4 Wk. Tropical |       |      |     |
|------------|---------------------------------------------------------------------------------------------------|------------|-------|------|----------------|-------|------|-----|
|            |                                                                                                   | 10/i Speed | Gamma | Fog  | 10/i Speed     | Gamma | Fog  |     |
| 12         | Control                                                                                           | None       | 1,180 | 1.24 | .06            | 780   | 1.07 | .22 |
| 13         | do                                                                                                | None       | 980   | 1.29 | .07            | 460   | 1.30 | .22 |
| 14         | Pd(C <sub>2</sub> H <sub>5</sub> NH <sub>2</sub> ) <sub>2</sub> Cl <sub>2</sub>                   | 1.5        | 1,100 | 1.20 | .06            | 940   | 1.14 | .08 |
| 15         | Pd(C <sub>5</sub> H <sub>4</sub> N) <sub>2</sub> Cl <sub>2</sub>                                  | 1.0        | 1,080 | 1.24 | .07            | 1,080 | 1.23 | .11 |
| 16         | Pd             | 1.0        | 1,000 | 1.30 | .07            | 1,120 | 1.16 | .13 |
| 17         | Pd(C <sub>2</sub> H <sub>5</sub> CH <sub>2</sub> NH <sub>2</sub> ) <sub>2</sub> Cl <sub>2</sub>   | 1.0        | 1,120 | 1.17 | .05            | 1,200 | 1.18 | .10 |
| 18         | Control                                                                                           | None       | 1,850 | 1.39 | .21            | 1,120 | 0.96 | .35 |
| 19         | do                                                                                                | None       | 2,200 | 1.28 | .22            | 1,400 | 1.00 | .30 |
| 20         | Pd(C <sub>2</sub> H <sub>4</sub> ) <sub>2</sub> Cl <sub>2</sub>                                   | 0.25       | 1,850 | 1.46 | .16            | 1,750 | 0.91 | .28 |
| 21         | Pd(H <sub>2</sub> N-C <sub>2</sub> H <sub>4</sub> -NH <sub>2</sub> ) <sub>2</sub> Cl <sub>2</sub> | 0.25       | 2,000 | 1.23 | .20            | 1,320 | 0.95 | .38 |

and upon the specific complex salt used as a stabilizer and fog inhibitor.

The anti-foggant and stabilizing action was determined by incubation of the emulsions under simulated tropical conditions and also by incubation at low relative humidity at 120° F. for various lengths of time from 12 days to one month. The results of these tests are tabulated here and are compared with the initial speed, gamma and fog of the emulsions with and without the anti-foggant and stabilizing compound. The tests from which the following tabulation was made

65 It will be apparent from the above data that, considering all of the stabilizing compounds of our invention, the palladous halide complexes of ammonia, the heterocyclic tertiary nitrogen compounds and ethylene are the most effective compounds for stabilizing both speed and fog of emulsions and of these three preferred groups of complexes, the ammonia complexes appear to be most effective, the heterocyclic tertiary nitrogen complexes next, and the ethylene complexes least effective since the latter tend to inhibit fog less.

One of the advantages of our invention is the fact that the compounds are readily prepared with high purity. The compounds are prepared by the methods shown in the Textbook of Inorganic Chemistry by M. M. J. Sutherland, published by Charles Griffin and Company, Ltd., London, vol. 10, pages 193 to 243 (1928). For example, diamminepalladous chloride is prepared by the addition of concentrated aqueous ammonia to an aqueous palladous chloride solution until the precipitate first formed just dissolves. The solution is then evaporated to dryness, extracted with water and heated slightly to remove excess ammonia. After cooling and acidifying with excess concentrated hydrochloric acid, the product is allowed to crystallize. The resultant yellow crystalline powder is then washed with a limited quantity of water and dried at 100° C.

The iodo compound prepared as above is less soluble in water but nevertheless gives satisfactory results as an antifoggant at concentrations of the order shown in the above table. The other palladium compounds of the invention are prepared and used in an analogous manner.

The fog inhibiting agents which we have described may be used in various kinds of photographic emulsions. In addition to being useful in ordinary non-sensitized emulsions they may also be used in orthochromatic, panchromatic and X-ray emulsions. If used with sensitizing dyes, they may be added to the emulsion before or after the dyes are added. Various silver salts may be used as the sensitive salt such as silver bromide, silver iodide, silver chloride and mixtures of these. The dispersing agents may be gelatin or other colloid such as collodion, albumen, cellulose organic derivatives or synthetic resins.

We also contemplate as a part of our invention those cases where it is desirable to coat the antifoggant in a colloid layer such as gelatin on either or both sides of or also in a silver halide emulsion layer, so that the antifoggant is contiguous to the silver halide emulsion. In these cases we use the same or a slightly greater ratio of rare metal salt to silver halide as when the salt is in the emulsion layer.

It will be understood that we contemplate as included within our invention all modifications and equivalents falling within the scope of the appended claims.

We claim:

1. A photographic silver halide emulsion containing an acido-palladium complex as a stabilizing agent.
2. A photographic silver halide emulsion containing as a stabilizing agent a dipyrnidiniumpalladous halide.
3. A photographic silver halide emulsion containing as a stabilizing agent, dipyrnidiniumpalladous chloride.
- 10 4. A photographic silver halide emulsion containing as a stabilizing agent, an acido-diammine-palladium complex.
- 15 5. A photographic silver halide emulsion containing as a stabilizing agent, a diamminepalladous halide.
6. A photographic silver halide emulsion containing as a stabilizing agent, diamminepalladous chloride.
- 20 7. A photographic silver halide emulsion containing as a stabilizing agent, a diethylenepalladous halide.
8. A photographic silver halide emulsion containing as a stabilizing agent, diethylenepalladous chloride.
- 25 9. A light-sensitive photographic element comprising a silver halide emulsion layer and an organic colloid layer contiguous to said emulsion layer, at least one of said layers containing an acido-diammine-palladium complex as a stabilizing agent for said emulsion layer.
- 30 10. A photographic silver halide emulsion containing as a stabilizing agent an acido-palladium complex containing in the cation a palladium atom and a basic nitrogen atom.
- 35 11. A photographic silver halide emulsion containing as a stabilizing agent an acido-palladium complex containing in the cation a palladium atom and a basic nitrogen atom of a heterocyclic ring compound.

ROBERT E. STAUFFER.  
WILLIAM F. SMITH.

#### REFERENCES CITED

45 The following references are of record in the file of this patent:

#### UNITED STATES PATENTS

| Number       | Name               | Date          |
|--------------|--------------------|---------------|
| 2,448,060    | Smith et al. _____ | Aug. 31, 1948 |
| 50 2,448,857 | Brice _____        | Sept. 7, 1948 |